



US008863490B2

(12) **United States Patent**  
**Boisseau et al.**

(10) **Patent No.:** **US 8,863,490 B2**  
(45) **Date of Patent:** **Oct. 21, 2014**

(54) **MULTI-STRAND CORD IN WHICH THE BASIC STRANDS ARE DUAL LAYER CORDS, RUBBERIZED IN SITU**

(75) Inventors: **Sandra Boisseau**, Chappes (FR); **Henri Barguet**, Martres-d'Artiere (FR); **Thibaud Pottier**, Clermont-Ferrand (FR)

(73) Assignees: **Michelin Recherche et Techniques S.A.**, Granges-Paccot (CH); **Compagnie Generale des Etablissements Michelin**, Clermont-Ferrand (FR)

(\*) Notice: Subject to any disclaimer, the term of this patent is extended or adjusted under 35 U.S.C. 154(b) by 358 days.

(21) Appl. No.: **13/382,150**

(22) PCT Filed: **Jul. 5, 2010**

(86) PCT No.: **PCT/EP2010/059524**

§ 371 (c)(1),  
(2), (4) Date: **Mar. 22, 2012**

(87) PCT Pub. No.: **WO2011/000963**

PCT Pub. Date: **Jan. 6, 2011**

(65) **Prior Publication Data**

US 2012/0174557 A1 Jul. 12, 2012

(30) **Foreign Application Priority Data**

Jul. 3, 2009 (FR) ..... 09 54592

(51) **Int. Cl.**

**D02G 3/48** (2006.01)  
**D07B 1/16** (2006.01)  
**D07B 1/06** (2006.01)  
**D07B 7/14** (2006.01)

(52) **U.S. Cl.**  
CPC ..... **D07B 1/0613** (2013.01); **D07B 2205/306** (2013.01); **D07B 2201/2046** (2013.01);

(Continued)

(58) **Field of Classification Search**  
CPC .... **D07B 1/0606**; **D07B 1/062**; **D07B 1/0626**; **B60C 9/0007**; **B60C 2015/0685**  
USPC ..... **57/211, 212, 223, 232, 237, 241**  
See application file for complete search history.

(56) **References Cited**

U.S. PATENT DOCUMENTS

5,139,874 A \* 8/1992 Starinshak et al. ..... 428/375  
5,279,695 A \* 1/1994 Starinshak et al. ..... 156/296

(Continued)

FOREIGN PATENT DOCUMENTS

FR 2 925 922 7/2009  
FR 2 925 923 7/2009

(Continued)

*Primary Examiner* — Shaun R Hurley

(74) *Attorney, Agent, or Firm* — Cozen O'Connor

(57) **ABSTRACT**

J strands form a core. K outer strands are wound around it in a helix with pitch  $P_K$ , each having a cord with an L wire inner layer of diameter  $d_1$ , and an M wire outer layer of diameter  $d_2$ , wound around the inner layer in a helix with pitch  $p_2$ ; with (in mm):  $0.10 < d_1 < 0.50$ ;  $0.10 < d_2 < 0.50$ ;  $6 < p_2 < 30$ ; its inner layer is sheathed with filling rubber; over any length  $P_K$  of the outer strand, filling rubber is in each of the capillaries delimited by L wires of the inner layer and M wires of the outer layer, and also, when L is equal to 3 or 4, in the central channel delimited by L wires of the inner layer. Filling rubber in said outer strand is 5 to 40 mg per g of strand.

**36 Claims, 6 Drawing Sheets**



## (52) U.S. Cl.

CPC ..... *D07B 1/0626* (2013.01); *D07B 2201/2062* (2013.01); *D07B 2205/3075* (2013.01); *D07B 2207/4072* (2013.01); *D07B 1/062* (2013.01); *D07B 2201/2032* (2013.01); *D07B 2201/2061* (2013.01); *D07B 2205/3067* (2013.01); ***D07B 1/165*** (2013.01); *D07B 2501/2046* (2013.01); *D07B 2201/2023* (2013.01); *D07B 2201/2011* (2013.01); *D07B 2205/3071* (2013.01); *D07B 2201/2065* (2013.01); *D07B 2201/1032* (2013.01); *D07B 2201/2059* (2013.01); *D07B 2201/1044* (2013.01); *D07B 2201/203* (2013.01); *D07B 2201/102* (2013.01); *D07B 2205/3021* (2013.01); *D07B 7/145* (2013.01); *D07B 2201/2039* (2013.01); *D07B 2201/2081* (2013.01); *D07B 2201/2028* (2013.01); *D07B 2205/3089* (2013.01)

USPC ..... **57/223**; 57/237; 57/241

## (56) References Cited

## U.S. PATENT DOCUMENTS

5,461,850 A \* 10/1995 Bruyneel et al. ..... 57/212  
 6,247,514 B1 \* 6/2001 Kim et al. ..... 152/556  
 6,360,522 B1 \* 3/2002 Walton ..... 57/212  
 6,817,395 B2 \* 11/2004 Sinopoli et al. ..... 152/527  
 6,863,103 B1 \* 3/2005 Masubuchi et al. ..... 152/451  
 7,458,200 B2 \* 12/2008 Kish ..... 57/237  
 8,117,818 B2 \* 2/2012 Ikehara ..... 57/237  
 8,191,348 B2 \* 6/2012 Barguet et al. ..... 57/223  
 8,209,949 B2 \* 7/2012 Barguet et al. ..... 57/212

8,601,782 B2 \* 12/2013 Nakamura ..... 57/218  
 8,627,696 B2 \* 1/2014 Pottier et al. ..... 72/64  
 2002/0160213 A1 \* 10/2002 Imamiya et al. ..... 428/465  
 2003/0106300 A1 \* 6/2003 Bruyneel et al. ..... 57/212  
 2005/0121126 A1 \* 6/2005 Hirachi et al. ..... 152/451  
 2007/0130905 A1 \* 6/2007 Kish ..... 57/237  
 2008/0318077 A1 \* 12/2008 Barguet et al. ..... 428/592  
 2009/0294009 A1 \* 12/2009 Barguet et al. ..... 152/527  
 2010/0000645 A1 \* 1/2010 Ikehara ..... 152/451  
 2010/0170215 A1 \* 7/2010 Nishimura ..... 57/258  
 2011/0011486 A1 \* 1/2011 Pottier et al. ..... 140/149  
 2011/0017376 A1 \* 1/2011 Pottier et al. ..... 152/451  
 2011/0198008 A1 \* 8/2011 Pottier et al. ..... 152/451  
 2011/0315296 A1 \* 12/2011 Cogne et al. ..... 152/556  
 2012/0000590 A1 \* 1/2012 Cogne et al. ..... 152/564  
 2012/0055602 A1 \* 3/2012 Nishimura ..... 152/451  
 2012/0159919 A1 \* 6/2012 Gauthier et al. ..... 57/212  
 2012/0174557 A1 \* 7/2012 Boisseau et al. ..... 57/213  
 2012/0285602 A1 \* 11/2012 Domingo et al. ..... 152/548  
 2012/0298276 A1 \* 11/2012 Barguet et al. ..... 152/527  
 2012/0298280 A1 \* 11/2012 Domingo ..... 152/556  
 2012/0318428 A1 \* 12/2012 Domingo ..... 152/556  
 2013/0199690 A1 \* 8/2013 Barguet et al. ..... 152/527  
 2013/0292027 A1 \* 11/2013 Sallaz et al. ..... 152/552  
 2013/0340913 A1 \* 12/2013 Sallaz et al. ..... 152/552  
 2014/0008003 A1 \* 1/2014 Sallaz et al. ..... 152/552

## FOREIGN PATENT DOCUMENTS

|    |                |        |
|----|----------------|--------|
| JP | 7 054286       | 2/1995 |
| JP | 2009 024268    | 2/2009 |
| WO | WO 2009/011397 | 1/2009 |
| WO | WO 2009/080583 | 7/2009 |
| WO | WO 2010/012411 | 2/2010 |

\* cited by examiner

**Fig. 1****Fig. 2**

**Fig. 3**

Fig. 4Fig. 5

**Fig. 6**

**Fig. 7**

Fig. 8

## 1

**MULTI-STRAND CORD IN WHICH THE  
BASIC STRANDS ARE DUAL LAYER CORDS,  
RUBBERIZED IN SITU**

RELATED APPLICATIONS

This is a U.S. National Phase Application under 35 USC §371 of International Application PCT/EP2010/059524, filed on Jul. 5, 2010.

This application claims the priority of French application Ser. No. 09/54592 filed on Jul. 3, 2009, the content of which is hereby incorporated by reference.

FIELD OF THE INVENTION

The present invention relates to very high-strength multi-strand cords (also called multistrand ropes), which can especially be used for the reinforcement of pneumatic tires for heavy industrial vehicles, such as civil engineering vehicles of the mining type.

The invention also relates to cords of the “rubberized in situ” type, that is to say coated on the inside, during their very manufacture, by rubber or a rubber composition in the uncrosslinked (green) state, before they are incorporated into rubber articles, such as tires, which they are intended to reinforce.

The invention also relates to tires and to the reinforcements for these tires, and to the crown reinforcements, also called “belts”, of these tires, and more particularly to the reinforcement of the tire belts for heavy industrial vehicles.

As is known, a radial tire comprises a tread, two inextensible beads, two sidewalls connecting the beads to the tread, and a belt placed circumferentially between the carcass reinforcement and the tread. This belt is made up of various rubber plies (or “layers”) which may or may not be reinforced by reinforcing elements (called “reinforcers”) such as cords or monofilaments, of the metal or textile type.

BACKGROUND OF THE INVENTION

The belt generally consists of several superposed belt plies, sometimes called “working” plies or “crossed” plies, the generally metallic reinforcing cords of which are placed so as to be practically parallel to one another within a ply but crossed from one ply to another, that is to say they are inclined, whether symmetrically or not, to the median circumferential plane. These crossed plies are generally accompanied by various other auxiliary rubber plies or layers, which vary in width depending on the case and may or may not comprise metal reinforcers. Mention may in particular be made of what are called “protective” plies responsible for protecting the rest of the belt from external attack, from perforations, or else what are called “hoop” plies having metallic or non-metallic reinforcers oriented substantially in the circumferential direction, (so-called “zero-degree” plies), irrespective of whether they are radially outer or inner in relation to the crossed plies.

As is known, such a tire belt must meet various, often contradictory, requirements, in particular:

it must be as rigid as possible at low deformation, as it contributes substantially to stiffening the tire crown; it must have as low a hysteresis as possible, in order, on the one hand, to minimize heating of the inner region of the crown during running and, on the other hand, to reduce the rolling resistance of the tire, this being synonymous with fuel economy; and; finally, it must have a high endurance, in particular with respect to the phenomenon of separation, cracking of the

## 2

ends of the crossed plies in the shoulder region of the tire, known as “cleavage”, which in particular requires metal cords that reinforce the belt plies to have a high compressive fatigue strength, when in a relatively corrosive atmosphere.

The third requirement is particularly important in the case of tires for industrial vehicles, such as heavy goods vehicles or civil engineering machinery, which are designed in particular to be able to be retreaded one or more times when their treads reach a critical stage of wear after prolonged running or usage.

To reinforce the working crown plies of the belts of such above tires, it is general practice to use two-layer multistrand steel cords consisting of a core comprising J strands forming an inner layer (Ci), J typically varying from 1 to 4, around which core are helically wound, with a helix pitch  $P_K$ , K outer strands forming an outer layer (Ce) around said inner layer (Ci), as described for example in the patents or patent applications U.S. Pat. No. 5,461,850, U.S. Pat. No. 5,768,874, U.S. Pat. No. 6,247,514, U.S. Pat. No. 6,817,395, U.S. Pat. No. 6,863,103, U.S. Pat. No. 7,426,821, US 2007/0144648 and WO 2008/026271.

As is well known by those skilled in the art, these multi-strand cords must be impregnated as much as possible by the rubber in the tire belts that they reinforce, so that this rubber penetrates as much as possible into spaces between the wires constituting the strands. If this penetration is insufficient, empty channels then remain along the strands, and corrosive agents, for example water, capable of penetrating the tires, for example as a result of the tire belt being cut or otherwise attacked, travel along these channels through said belt. The presence of this moisture plays an important role, causing corrosion and accelerating the fatigue process (so-called “fatigue-corrosion” phenomena) compared to use in a dry atmosphere.

All these fatigue phenomena, generally grouped together under the generic term “fatigue-fretting corrosion”, are the cause of progressive degeneration of the mechanical properties of the cords and strands and may, under the most severe running conditions, affect the lifetime of the latter.

Moreover, it is known that good penetration of the cord by rubber makes it possible, because of the small volume of air trapped in the cord, to reduce the cure time of the tires (shortened “in-press time”).

However, the constituent elementary strands of these multistrand cords have, at least in certain cases, the drawback of not being able to be penetrated right to the core.

This is in particular the case for elementary strands of 3+M or 4+M construction, because of the presence of a channel or capillary at the centre of the three core wires, which remains empty after external impregnation with rubber and therefore propitious, through a kind of “wicking” effect, to the propagation of corrosive media such as water. This drawback of the strands of 3+M construction is well known; it has been explained for example in the patent applications WO 01/00922, WO 01/49926, WO 2005/071157 and WO 2006/013077.

To solve this problem of penetrability right to the core of cords of 3+M construction, patent application US 2002/160213 has certainly proposed producing strands of the type rubberized in situ. The process proposed here consists in sheathing, individually (i.e. in isolation, “wire to wire”) with rubber in the uncured state, upstream of the point of assembly (or twisting point) of the three wires, just one or preferably each of the three wires in order to obtain a rubber-sheathed

inner layer before the M wires of the outer layer are subsequently put in place by being corded around the inner layer thus sheathed.

The above application provides no information relating to the construction of the 3+M strands, in particular neither information about the assembly pitches nor information about the amounts of filing rubber to be used. Furthermore, the proposed process poses many problems.

Firstly, the sheathing of one single wire in three (as illustrated for example in FIGS. 11 and 12 of this patent application US 2002/160213) does not guarantee sufficient filling of the final strand with the rubber and therefore prevents satisfactory corrosion resistance being obtained. Secondly, the wire-to-wire sheathing of each of the three wires (as illustrated for example in FIGS. 2 and 5 of that document), although effectively filling the strand, leads to the use of an excessively large amount of rubber. The overspill of rubber at the periphery of the final strand then becomes unacceptable under industrial cabling and rubber-coating conditions.

Because of the very high adhesion of rubber in the green (i.e. uncrosslinked) state, the strand thus rubberized becomes unusable because of the undesirable adhesion to the manufacturing tools or between the strand turns during winding of the latter onto a take-up reel, without even mentioning the final impossibility of correctly calendering the cord. It will be recalled here that calendering consists in converting the cord, by incorporation between two layers of rubber in the green state, into a rubberized metal fabric serving as semi-finished product for any subsequent manufacture, for example to produce a tire.

Another problem posed by the insulated sheathing of each of the three wires is the large amount of space required by using three extrusion heads. Because of such a space requirement, the manufacture of cords having cylindrical layers (i.e. with different pitches  $p_1$  and  $p_2$  from one layer to another, or with identical pitches  $p_1$  and  $p_2$  but with different twisting directions from one layer to the other) must necessarily be carried out in two batch operations: (i) individual sheathing of the wires followed by cabling and winding of the inner layer in a first step; and (ii) cabling of the outer layer around the inner layer in a second step. Again because of the high adhesion of rubber in the green state, the winding and intermediate storage of the inner layer require the use of spacers and many separators during winding onto an intermediate reel, so as to avoid undesirable adhesion between the coiled layers or between the turns of a given layer.

All the above constraints are greatly prejudicial from the industrial standpoint and in conflict with the aim of producing high manufacturing rates.

## SUMMARY OF THE INVENTION

By continuing their research, the Applicants have discovered a novel two-layer multistrand cord of J+K construction, the K outer strands of which, thanks to a specific structure obtained according to one particular manufacturing process, make it possible to alleviate the aforementioned drawbacks.

Consequently, a first aspect of the invention is directed to a multistrand metal cord having two layers of J+K construction, which can especially be used for reinforcing tires for industrial vehicles, consisting of a core comprising J strands forming an inner layer, J varying from 1 to 4, around which core are wound, in a helix, with a helix pitch PK of between 20 and 70 mm, K outer strands forming an outer layer around said inner layer, each outer strand:

consisting of a cord having two layers (C1, C2) of L+M construction, rubberized in situ, comprising an inner

layer (C1) consisting of L wires of diameter  $d_1$ , L varying from 1 to 4, and an outer layer (C2) of M wires, M being equal to or greater than 5, of diameter  $d_2$ , which are wound together in a helix with a pitch  $p_2$  around the inner layer (C1); and

having the following characteristics ( $d_1$ ,  $d_2$  and  $p_2$  being expressed in mm):

$0.10 < d_1 < 0.50$ ;

$0.10 < d_2 < 0.50$ ;

$6 < p_2 < 30$ ;

its inner layer (C1) is sheathed with a rubber composition called a "filling rubber";

over any length of the outer strand equal to  $P_K$ , the filling rubber is present in each of the capillaries delimited by the L wires of the inner layer (C1) and the M wires of the outer layer (C2), and also, when L is equal to 3 or 4, in the central channel delimited by the L wires of the inner layer (C1); and

the amount of filling rubber in said outer strand is between 5 and 40 mg per g of strand.

Such a multistrand cord can be used for reinforcing rubber articles or semi-finished products, for example plies, hoses, belts, conveyor belts and tires.

The multistrand cord of the invention is most particularly intended for use as reinforcing element for a belt of a tire intended for industrial vehicles, such as "heavy" vehicles, i.e. underground trains, buses, road transport vehicles (lorries, tractors, trailers), off-road vehicles, and agricultural or civil engineering machinery and other transport or handling vehicles.

Another aspect of the invention relates to these rubber articles or semi-finished products themselves when they are reinforced with a multistrand cord according to the invention, particularly tires intended especially for industrial vehicles.

## BRIEF DESCRIPTION OF THE DRAWINGS

The invention and its advantages will be readily understood in the light of the description and the embodiments that follow, together with FIGS. 1 to 8 which relate to these embodiments and which schematically show, respectively:

in cross section, a strand of 3+9 construction, of the type having cylindrical layers, which can be used in the multistrand cord according to an embodiment of the invention (FIG. 1);

in cross section, a strand of 3+9 construction, of the type having cylindrical layers, which can be used in the multistrand cord of the invention (FIG. 1);

in cross section, an example of a multistrand cord according to the invention, of (1+6)×(3+9) construction, incorporating the strand of FIG. 1 (FIG. 2);

in cross section, another example of a multistrand cord according to the invention, of (1+6)×(3+9) construction, incorporating the strand of FIG. 1 (FIG. 3);

in cross section, another example of a strand of 3+9 construction, of compact type, which can be used in the multistrand cord of the invention (FIG. 4);

in cross section, another example of a multistrand cord according to the invention, of (1+6)×(3+9) construction, incorporating the strand of FIG. 4 (FIG. 5);

in cross section, another example of a multistrand cord according to the invention, of (1+6)×(3+9) construction, incorporating the strand of FIG. 4 (FIG. 6);

an example of an installation for twisting and in situ rubberizing, which can be used for producing strands intended for the manufacture of the multistrand cord of the invention (FIG. 7); and

in radial cross section, a tire casing for an industrial vehicle with a radial carcass reinforcement, whether or not in accordance with the invention in this general representation (FIG. 8).

## I. MEASUREMENTS AND TESTS

### I-1. Tensile Test Measurements

As regards the metal wires and cords, the measurements of the breaking force denoted by  $F_m$  (maximum load in N), the tensile strength denoted by  $R_m$  (in MPa) and the elongation at break denoted by  $A_e$  (total elongation in %) are carried out in tension according to the ISO 6892 (1984) standard.

As regards the diene rubber compositions, the modulus measurements are carried out in tension, unless otherwise indicated according to the ASTM D 412 (1998) standard (specimen "C"): the "true" secant modulus (i.e. referred to the actual cross section of the specimen) is measured in a second elongation (i.e. after an accommodation cycle) with a 10% elongation, the modulus being denoted by E10 and expressed in MPa (under the normal temperature and relative humidity conditions according to the ASTM D 1349 (1999) standard).

### I-2. Air Permeability Test

This test enables the longitudinal air permeability of the tested elementary cords to be determined by measuring the volume of air crossing through a specimen under constant pressure over a given time. The principle of such a test, well known to those skilled in the art, is to demonstrate the effectiveness of the treatment of a cord in order to make it impermeable to air. The test has been described for example in the standard ASTM D2692-98.

The test is carried out here either on strands extracted from multistrand cords as produced, having undergone subsequent coating and curing, or on cords extracted from tires or from the rubber plies that these multistrand cords reinforce, and therefore already coated with cured rubber.

In the first case (multistrand cords as produced), the extracted cords must, before the test, be coated from the outside with a rubber coating compound. To do this, a series of 10 strands arranged so as to be in parallel (with an inter-strand distance of 20 mm) is placed between two skims (two rectangles measuring 80×200 mm) of a cured rubber composition, each skim having a thickness of 3.5 mm. The whole assembly is then clamped in a mould, each of the strands being maintained under sufficient tension (for example 2 daN) to ensure that it remains straight when being placed in the mould, using clamping modules. The vulcanization (curing) process then takes place over 40 minutes at a temperature of 140° C. and under a pressure of 15 bar (rectangular piston measuring 80×200 mm), after which the assembly is demoulded and cut up into 10 specimens of metal strands thus coated, in the form of parallelepipeds measuring 7 mm×7 mm×L<sub>t</sub> for characterization.

A conventional tire rubber composition is used as rubber coating compound, said composition being based on natural (peptized) rubber and N330 carbon black (65 phr) and also containing the following standard additives: sulphur (7 phr); sulphonamide accelerator (1 phr); ZnO (8 phr); stearic acid (0.7 phr); antioxidant (1.5 phr); and cobalt naphthenate (1.5 phr). The modulus E10 of the rubber coating compound is about 10 MPa.

The test is carried out on a predetermined length L<sub>t</sub> (for example equal to P<sub>K</sub>, 3 cm or even 2 cm), thus coated with its surrounding rubber composition (or rubber coating com-

pound), in the following manner: air under a pressure of 1 bar is injected into the inlet of the strand and the volume of air leaving it is measured using a flowmeter (calibrated for example from 0 to 500 cm<sup>3</sup>/min). During the measurement, the strand specimen is immobilized in a compressed seal (for example a rubber or dense foam seal) in such a way that only the amount of air passing through the strand from one end to the other, along its longitudinal axis, is measured. The sealing capability of the seal is checked beforehand using a solid rubber specimen, that is to say one without strands.

The measured average air flow rate (the average over the 10 specimens) is lower the higher the longitudinal impermeability of the strand. Since the measurement is accurate to ±0.2 cm<sup>3</sup>/min, measured values of 0.2 cm<sup>3</sup>/min or less are considered to be zero—they correspond to a strand that can be termed airtight (completely airtight) along its axis (i.e. in its longitudinal direction).

### I-3. Amount of Filling Rubber

The amount of filling rubber is measured by difference between the weight of the initial strand (therefore in situ rubberized) and the weight of the strand (and therefore that of its wires) from which the filling rubber has been removed by an appropriate electrolytic treatment.

A strand specimen (1 m in length), wound on itself to reduce its space requirement, constitutes the cathode of an electrolyzer (connected to the negative terminal of a generator), whereas the anode (connected to the positive terminal) consists of a platinum wire. The electrolyte consists of an aqueous solution (demineralized water) containing 1 mol per liter of sodium carbonate.

Voltage is applied to the specimen, completely immersed in the electrolyte, for 15 min under a current of 300 mA. Next, the strand is removed from the bath and rinsed copiously with water. This treatment allows the rubber to be easily detached from the strand (if this is not so, the electrolysis is continued for a few minutes). The rubber is carefully removed, for example by simply wiping using an absorbant cloth, while untwisting the wires of the strand one by one. The wires are again rinsed with water and then immersed in a beaker containing a demineralized water (50%)/ethanol (50%) mixture. The beaker is immersed in an ultrasonic bath for 10 minutes. The wires thus stripped of any trace of rubber are removed from the beaker, dried in a stream of nitrogen or air, and finally weighed.

Deduced therefrom, by calculation, is the amount of filling rubber in the strand, expressed in mg (milligrams) of filling rubber per g (gram) of initial strand, and averaged over 10 measurements (i.e. along 10 meters of strand in total).

## II. DETAILED DESCRIPTION

In the present description, unless expressly indicated otherwise, all the percentages (%) indicated are percentages by weight.

Moreover, any interval of values denoted by the expression "between a and b" represents the range of values going from more than a to less than b (i.e. the limits a and b are excluded) whereas any interval of values denoted by the expression "from a to b" means the range of values going from a up to b (i.e. the strict limits a and b are included).

### II-1. Multistrand Cord of the Invention

The multistrand metal cord of the invention therefore consists of a core (i.e., as a reminder, the supporting member for

the outer layer) comprising J strands forming an inner layer (Ci), J varying from 1 to 4, around which core are wound in a helix, with a helix pitch  $P_K$  of between 20 and 70 mm, K outer strands forming an outer layer (Ce) around said inner layer (Ci).

Each of the K outer strands itself consists of a cord having two layers (C1, C2) of L+M construction, rubberized in situ, comprising an inner layer (C1) consisting of L wires of diameter  $d_1$ , L varying from 1 to 4, and an outer layer (C2) of M wires, M being equal to or greater than 5, of diameter  $d_2$ , which are wound together in a helix with a pitch  $p_2$  around the inner layer (C1).

Each of these K outer strands furthermore has the following characteristics ( $d_1$ ,  $d_2$  and  $p_2$  being expressed in mm):

$$0.10 < d_1 < 0.50;$$

$$0.10 < d_2 < 0.50;$$

$$6 < p_2 < 30;$$

its inner layer (C1) is sheathed with a rubber composition called a "filling rubber";

over any length of the outer strand equal to  $P_K$ , the filling rubber is present in each of the capillaries bounded by the L wires of the inner layer (C1) and the M wires of the outer layer (C2), and also, when L is equal to 3 or 4, in the central channel bounded by the L wires of the inner layer (C1); and

the amount of filling rubber in said outer strand is between 5 and 40 mg per g of outer strand.

Each outer strand may thus be termed an in situ rubberized cord, that is to say rubberized on the inside, during its very manufacture (therefore in the as-manufactured state), with the filling rubber. In other words, each of the capillaries or interstices (these two terms are interchangeable, denoting the voids or free spaces where there is no filling rubber) that are located between and delimited by the wires of the inner layer (C1) and the wires of the outer layer (C2) is at least partly filled, whether continuously or not, along the axis of strand, with the filling rubber. Furthermore, the central channel or capillary formed by the 3 or 4 wires of the inner layer C1, when L is equal to 3 or 4, also penetrated by some filling rubber.

According to a preferred embodiment, over any outer strand portion equal to  $P_K$  (more preferably equal to 3 cm, even more preferably equal to 2 cm), the central channel (when L is equal to 3 or 4) and each capillary or interstice, as described above, comprise at least one rubber plug. In other words, and preferably, there is at least one rubber plug every  $P_K$  (more preferably every 3 cm, more preferably still every 2 cm of outer strand), which obstructs the central channel and each capillary or interstice of the outer strand in such a way that, in the air permeability test (according to section I-2), each outer strand of the multistrand core of the invention has an average air flow rate of less than 2  $\text{cm}^3/\text{min}$ , more preferably less than or at most equal to 0.2  $\text{cm}^3/\text{min}$ .

Each outer strand has, as essential other feature, the fact that its amount of filling rubber is between 5 and 40 mg of rubber compound per g of strand.

Below the minimum indicated, it is not possible to guarantee that, over any length of the outer strand length equal to  $P_K$  (more preferably equal to 3 cm, even more preferably equal to 2 cm), the filling rubber is in fact present, at least in part, in each of the interstices or capillaries of the outer strand, whereas, above the indicated maximum, the various problems described previously due to the overspill of filling rubber at the periphery of the strand are encountered. For all these reasons, it is preferable for the amount of filling rubber to be between 5 and 35 mg, more preferably still in the range from 10 to 30 mg per g of strand.

Such an amount of filling rubber, this being controlled within the abovementioned limits, is made possible only by virtue of the use of a specific twisting-rubberizing process adapted to the geometry of each outer strand of L+M construction, which process will be explained in detail subsequently.

The implementation of this specific process, while enabling a strand to be obtained in which the amount of filling rubber is controlled, guarantees the presence of internal partitions (continuous or discontinuous along the axis of the strand) or rubber plugs in each outer strand, especially in its central channel when L is equal to 3 or 4, in sufficient number. Thus, each outer strand becomes impermeable to the propagation, along the strand, of any corrosive fluid, such as water or oxygen of air, thus eliminating the wicking effect described in the introduction of the present document.

According to one particularly preferred embodiment of the invention, the specific feature is verified: over any length of the outer strand equal to  $P_K$  (more preferably equal to 3 cm, even more preferably equal to 2 cm), each outer strand is airtight or almost airtight in the longitudinal direction.

In the air permeability test described in section I-2, an "airtight" L+M outer strand is characterized by an average air flow rate of less than or at most equal to 0.2  $\text{cm}^3/\text{min}$ , whereas an "almost airtight" L+M outer strand is characterized by an average air flow rate of less than 2  $\text{cm}^3/\text{min}$ , preferably less than 1  $\text{cm}^3/\text{min}$ .

For an optimized compromise between strength, feasibility, rigidity and endurance in compression of the cord, it is preferred for the diameters of the wires of the layers C1 and C2, which may or may not be the same from one layer to the other, to be between 0.15 and 0.35 mm.

The wires of the layers C1 and C2 may have the same diameter or a different diameter going from one layer to the other. It is possible to use wires of the same diameter from one layer to the other (i.e.  $d_1=d_2$ ), thereby simplifying in particular the manufacture of the strands and reducing their cost.

According to a preferred embodiment, in each outer strand,  $p_2$  is in the range from 12 to 25 mm.

According to another preferred embodiment,  $P_K$  is in the range from 25 to 60 mm, more preferably from 30 to 50 mm.

It will be recalled here that, as is known, the pitch "p" represents the length, measured parallel to the axis of the outer strand or of the multistrand cord, at the end of which a wire or an outer strand, respectively, having this pitch, completes one revolution about said axis.

Moreover, the following relationship is preferably satisfied:

$$1.5 \leq P_K/p_2 \leq 3.0.$$

Even more preferably, the following relationship is satisfied:

$$2.0 \leq P_K/p_2 \leq 2.5.$$

According to a preferred embodiment, in each outer strand, L is equal to 1, i.e. a single wire constitutes the inner layer (C1) of each outer strand.

According to another possible embodiment, L is different from 1 and, in such a case, the L wires of diameter  $d_1$  are helically wound with a pitch  $p_1$  preferably satisfying the relationship:

$$20 < p_1/d_1 < 100,$$

more preferably the relationship:

$$25 < p_1/d_1 < 75.$$

According to another preferred embodiment, L is different from 1 and, in such a case, the following relationship is preferably satisfied:

$$0.5 \leq p_1/p_2 \leq 1.$$

More preferably, in such a case, in each outer strand,  $p_1$  is in the range from 6 to 30 mm, preferably in the range from 6 to 25 mm. According to another, more preferable, embodiment, in each outer strand,  $p_1$  is equal to  $p_2$ .

According to another preferred embodiment, each outer strand satisfies the following relationship:

$$0.7 \leq d_1/d_2 \leq 1.3,$$

even more preferably the following relationship:

$$0.8 \leq d_1/d_2 \leq 1.2.$$

According to another preferred embodiment of the invention, when L is different from 1, in each outer strand, the M wires of the outer layer (C2) are helically wound either with a different pitch, or in a different twist direction, or with both a different pitch and a different twist direction, compared to the L wires of the inner layer (C1).

It is especially the case for strands having cylindrical layers, as described for example in FIG. 1, in which the two layers C1 and C2 are wound in the same twist direction (S/S or Z/Z) but with a different pitch (i.e.  $p_1 \neq p_2$ ). In such cylindrically layered strands, the compactness is such that the cross section of each outer strand has a cylindrical contour and not a polygonal one.

However, according to another possible embodiment of the invention, in each outer strand, the M wires of the outer layer (C2) may be helically wound with the same pitch and in the same twist direction as the L wires of the inner layer (C1), when L is different from 1, so as to obtain an outer strand of the compact type (i.e. with a polygonal contour).

The outer layer C2 of each of the K outer strands is preferably a saturated layer, that is to say, by definition, there is not sufficient space in this layer to add thereto at least one  $(M_{max}+1)$ th wire of diameter  $d_2$ ,  $M_{max}$  representing the maximum number of wires that can be wound as one layer around the inner layer C1. This construction has the advantage of limiting the risk of the filling rubber overspilling at its periphery and of providing, for a given outer strand diameter, a higher strength.

Thus, the number M of wires may vary very widely depending on the particular embodiment of the invention, for example from 5 to 14 wires, it being understood that L may vary from 1 to 4 and that the maximum number  $M_{max}$  of wires will be increased if their diameter  $d_2$  is reduced in comparison with the diameter  $d_1$  of the L core wires, so as preferably to maintain the outer layer in a saturated state.

Thus, according to one possible preferred embodiment, in each of the K outer strands, L is equal to 1 and M is more preferably equal to 5, 6 or 7. In other words, each outer strand is chosen from the group of cords having 1+5, 1+6 and 1+7 constructions. In this case, M is more preferably equal to 6.

According to another preferred embodiment of the invention, in each of the K outer strands, L is equal to 2 and M is more preferably equal to 7, 8 or 9. In other words, each outer strand is chosen from the group of cords of 2+7, 2+8 and 2+9 constructions. In this case, M is more preferably equal to 8.

According to another preferred embodiment of the invention, in each of the K outer strands, L is equal to 3 and M is more preferably equal to 8, 9 or 10. In other words, each outer strand is chosen from the group of cords of 3+8, 3+9 and 3+10 constructions. In this case, M is more preferably equal to 9.

According to another preferred embodiment of the invention, in each of the K outer strands, L is equal to 4 and M is more preferably equal to 8, 9, 10 or 11. In other words, each outer strand is chosen from the group of cords of 4+8, 4+9, 4+10 and 4+11 constructions. In this case, M is more preferably equal to 9 or 10.

Among all the above preferred outer strands, the wires of the two layers (C1, C2) may have the same diameter (i.e.  $d_1 = d_2$ ) or different diameters (i.e.  $d_1 \neq d_2$ ) from one layer (C1) to the other (C2).

The outer strands of the multistrand cord of the invention, like all multilayer cords, may be of two types, namely of the compact type or of the cylindrically layered type.

Preferably, when L is different from 1, all the wires of the layers C1 and C2 are wound in the same twist direction, i.e. either in the S direction (S/S arrangement) or in the Z direction (Z/Z arrangement). Winding the layers C1 and C2 in the same direction advantageously makes it possible to minimize the rubbing between these two layers and therefore the wear of the wires that constitute them. Even more preferably, the two layers C1 and C2 are wound in the same direction (S/S or Z/Z) and with a different pitch ( $p_1 < p_2$ ) in order to obtain an outer strand of the cylindrically layered type, as shown for example in FIG. 1.

FIG. 1 shows schematically, in cross section perpendicular to the axis of the strand (assumed to be straight and at rest), an example of a preferred strand that can be used in the multistrand cord of the invention, having a 3+9 construction.

This strand (10) is of the cylindrically layered type, i.e. the wires (11, 12) of its inner and outer layers (C1, C2) are either wound with the same pitch ( $p_1 = p_2$ ) but in a different direction (S/Z or Z/S), or wound with a different pitch ( $p_1 \neq p_2$ ) whatever the twist direction (S/S or Z/Z or S/Z or Z/S). As is known, this type of construction has the consequence that the wires are arranged as two adjacent layers (C1 and C2) that are concentric and tubular, giving a strand (and its two layers) an external outline E (shown dotted) which is cylindrical and not polygonal.

This FIG. 1 shows that the filling rubber (14), while very slightly splaying the wires, at least partly fills (here, in this example, completely fills) the central channel (13) delimited by the three wires (11) of the inner layer (C1) and also each of the capillaries or interstices (15) (as an example, some of these are shown symbolically by a triangle) that are located between, on the one hand, the 3 wires (11) of the inner layer (C1) and the 9 wires (12) of the outer layer (C2).

According to a preferred embodiment, in each outer strand of L+M construction, the filling rubber extends continuously around the inner layer (C1) that it covers.

According to another preferred embodiment of the invention, in the multistrand cord of the invention, each of the J strands of the core, J varying from 1 to 4, itself consists of a two-layer cord of L+M construction which, furthermore, preferably satisfies the characteristics of the K outer strands that were described above.

According to another, more preferable embodiment of the invention, each of the J strands of the core (J varying from 1 to 4) has a construction identical to that of the K outer strands. However, the invention also applies to cases in which each of the J strands has a construction different from that of the K outer strands.

According to one particular and preferred embodiment, the multistrand cord of the invention comprises in total 6 strands, a central strand forming the core or inner layer (C<sub>i</sub>) and 5 outer strands forming the outer layer (C<sub>e</sub>), said cord for example having the more particular 1×(1+6)+5×(3+9) construction.

## 11

According to another particular and preferred embodiment, the multistrand cord of the invention comprises in total 7 strands, a central strand forming the core or inner layer (Ci) and 6 outer strands forming the outer layer (Ce), said cord having for example the more particular  $(1+6) \times (1+6)$  construction or  $(1+6) \times (3+9)$  construction.

FIG. 2 shows schematically, in cross section perpendicular to the axis of the cord (again supposed to be straight and at rest), a preferred example of such a multistrand cord (denoted by C-1) according to the invention, having a  $(1+6) \times (3+9)$  construction or, according to an equivalent nomenclature, a  $1 \times (3+9) + 6 \times (3+9)$  construction. In this example, each of the 7 outer strands, i.e. the central strand (J=1) like the 6 outer strands (K=6) that surround it, have the same  $(3+9)$  construction corresponding to the elementary strand (10) described above in FIG. 1. This multistrand cord of the invention, by virtue of its individual strands being rubberized in situ, is, as may be seen, highly penetrated by the filling rubber (14), thereby giving it improved fatigue-corrosion resistance.

According to another particular and preferred embodiment, the multistrand cord of the invention comprises in total 8 strands, a central strand forming the core or inner layer (Ci) and 7 outer strands forming the outer layer (Ce), said cord having for example the more particular  $1 \times (3+9) + 7 \times (1+6)$  construction.

According to another particular and preferred embodiment, the multistrand cord of the invention comprises in total 9 strands, a central strand forming the core or inner layer (Ci) and 8 outer strands forming the outer layer (Ce), said cord having for example the more particular  $1 \times (3+9) + 8 \times (1+6)$  or  $1 \times (4+10) + 8 \times (1+6)$  construction.

According to another particular and preferred embodiment, the multistrand cord of the invention comprises in total 10 strands, a central strand forming the core or inner layer (Ci) and 9 outer strands forming the outer layer (Ce), said cord having for example the more particular  $1 \times (3+9) + 9 \times (1+6)$  or  $1 \times (4+10) + 9 \times (1+6)$  construction.

According to another particular and preferred embodiment, the multistrand core of the invention comprises in total 11 strands, 3 central strands forming the core or inner layer (Ci) and 8 outer strands forming the outer layer (Ce), said cord having for example the more particular  $3 \times (1+6) + 8 \times (1+6)$  or  $3 \times (3+9) + 8 \times (3+9)$  construction.

According to another particular and preferred embodiment, the multistrand cord of the invention comprises in total 12 strands, three central strands forming the core or inner layer (Ci) and 9 outer strands forming the outer layer (Ce), said cord having for example the more particular  $(3+9) \times (1+6)$  or  $(3+9) \times (3+9)$  construction.

According to another particular and preferred embodiment, the multistrand cord of the invention comprises in total 13 strands, 4 central strands forming the core or inner layer (Ci) and 9 outer strands forming the outer layer (Ce), said cord having for example the more particular  $4 \times (1+6) + 9 \times (1+6)$  or  $4 \times (3+9) + 9 \times (3+9)$  construction.

According to another particular and preferred embodiment, the multistrand cord of the invention comprises in total 14 strands, three central strands forming the core or inner layer (Ci) and 11 outer strands forming the outer layer (Ce), said cord having for example the more particular  $3 \times (3+9) + 11 \times (1+6)$  construction.

According to another particular and preferred embodiment, the multistrand cord of the invention comprises in total 15 strands, three central strands forming the core or inner layer (Ci) and 12 outer strands forming the outer layer (Ce), said cord having for example the more particular  $3 \times (3+9) + 12 \times (1+6)$  construction.

## 12

The multistrand cord of the invention may, according to one particularly preferred embodiment of the invention, comprise a core (as a reminder, consisting of the J strands, J varying from 1 to 4) which is itself sheathed with filling rubber in the unvulcanized state, this filling rubber having a formulation identical to or different from that used for the in situ rubberizing of the outer strands. To do this, as schematically illustrated in FIG. 7 for the constituent outer strands of the cord of the invention, it suffices to pass the core or inner layer (Ci) of the multistrand cord through an extrusion head of appropriate dimensions before the outer layer (Ce) of the K outer strands is put in place by cabling.

FIG. 3 shows schematically, in cross section perpendicular to the axis of the multistrand cord (assumed to be straight and at rest), an example of a multistrand cord (denoted by C-2) according to the invention, having a  $(1+6) \times (3+9)$  construction, in which the single central strand of  $(3+9)$  construction forming its inner layer Ci has itself been sheathed beforehand with filling rubber (16) before the 6 outer strands of  $(3+9)$  construction have been cabled around the central strand thus sheathed, in order to form the cylindrical outer layer Ce. It should be noted that the 7 outer strands (10) making up this cord C-2 are themselves rubberized in situ with filling rubber (14).

This multistrand cord of the invention, by virtue as it were of the "dual" in situ rubberizing, namely that of the individual strands during their prior manufacture and its own during the cabling thereof, shows, as may be seen, even better penetration by the filling rubber (14, 16), this being an indicator, recognized by those skilled in the art, of excellent fatigue-corrosion resistance.

The filling rubber (16) used for sheathing the core (consisting of J central strands, J varying from 1 to 4) of the multistrand cord of the invention may have a formulation identical to or different from the formulation of the filling rubber (14) used for the in situ rubberizing of the K outer strands.

The multistrand cords of the invention, like the strands described above that make up said cords, may be of two types, namely of the compact type or more preferably of the cylindrically layered type. They may or may not be provided with an outer wrap consisting of a single fine wire wound helically around the K outer strands in a direction (S or Z) identical or opposite to that of said outer strands.

FIG. 4 shows schematically, in cross section perpendicular to the axis of the strand (assumed to be straight and at rest), another example of a preferred strand that can be used in the multistrand cord of the invention, having a  $(3+9)$  construction.

This strand (20) is of the compact type, that is to say the wires (21, 22) of its inner and outer layers (C1, C2) are wound with the same pitch ( $p_1$  equals  $p_2$ ) and in the same direction (S/S or Z/Z). This type of construction has the consequence that the wires are arranged as two concentric and adjacent layers (C1 and C2) giving the strand (and its two layers) an external outline E (shown dotted) which is polygonal and not cylindrical.

FIG. 4 shows that the filling rubber (24), while very slightly splaying the wires, at least partly fills (here, in this example, completely fills) the central channel (23) delimited by the three wires (21) of the inner layer (C1) and each of the capillaries or interstices (25) (as an example, some of them have been shown symbolically by a triangle) that are located, on the one hand, between the 3 wires (21) of the inner layer (C1) and the 9 wires (22) of the outer layer (C2), these wires

## 13

being taken 3 by 3. In total 12 capillaries (25) are thus present in this strand, to which capillaries the central channel is added.

FIG. 5 shows schematically, in cross section perpendicular to the axis of the cord (again assumed to be straight and at rest), another preferred example of a multistrand cord (denoted by C-3) according to the invention, having a  $1 \times (1+6) + 6 \times (3+9)$  construction. In this example, each of the 6 outer strands has the same (3+9) construction corresponding to the strand (20) described previously with reference to FIG. 4. The central strand forming the core of the multistrand cord of the invention has a different construction, namely (1+6). This multistrand cord of the invention, by virtue of the in situ rubberizing of all of its individual strands, shows, as may be seen, great penetration by the filling rubber (24), thereby giving it a high fatigue-corrosion resistance.

FIG. 6 shows schematically another example of a multistrand cord (denoted by C-4) according to the invention, having a  $1 \times (1+6) + 6 \times (3+9)$  construction, identical to that of the previous cord C-3, but in which the single central strand of (1+6) construction forming its inner layer Ci has itself been sheathed beforehand with filling rubber (26) before the 6 outer strands of (3+9) construction have been cabled around the central strand thus sheathed, in order to form the cylindrical outer layer Ce. The 6 outer strands (10) making up this cord C-4 are rubberized in situ by filling rubber (14).

When J is different from 1, the strands of the inner layer Ci are preferably wound (with a helix pitch  $P_J$ ) in the same twist direction, i.e. either in the S direction (final S/S arrangement) or in the Z direction (final Z/Z arrangement), as those of the outer layer Ce. Winding the layers Ci and Ce in the same direction advantageously makes it possible to minimize the rubbing between these two layers and therefore the wear of the elementary strands that they constitute.

More preferably still, the two layers are wound in the same direction (S/S or Z/Z) and with a different pitch (preferably with  $P_J < P_K$ ), to obtain a multistrand cord of the cylindrically layered type, as shown for example in FIGS. 2 and 3.

Preferably, in the multistrand cord of the invention, when J is different from 1, the pitch  $P_J$  is between 15 and 45 mm, more preferably between 20 and 40 mm.

According to another preferred embodiment, when J is different from 1, the following relationship is satisfied:

$$0.5 \leq P_J / P_K \leq 1.$$

The invention relates of course to the multistrand cords described above both in the uncured state (their filling rubber then not being vulcanized) and in the cured state (their filling rubber then being vulcanized). However, it is preferred to use the multistrand cord of the invention with a filling rubber in the uncured state until it is subsequently incorporated into the semi-finished product or the finished product such as a tire for which it is intended, so as to promote bonding during the final vulcanization between the filling rubber and the surrounding rubber matrix (for example the calendering rubber).

The expression "metal cord or strand" is understood by definition in the present application to mean a cord or strand formed of wires consisting predominantly (i.e. more than 50% by number of these wires) or entirely (100% of the wires) of a metallic material. The wires are preferably made of steel, more preferably carbon steel. However, it is of course possible to use other steels, for example stainless steel, or other alloys.

When a carbon steel is used, its carbon content (% by weight of steel) is preferably between 0.4% and 1.2%, especially between 0.5% and 1.1%. These contents represent a good compromise between the mechanical properties

## 14

required of the tire and the feasibility of the wires. It should be noted that a carbon content between 0.5% and 0.6% makes such steels finally less expensive as they are easier to draw. Another advantageous embodiment of the invention may also consist, depending on the intended applications, in the use of steels having a low carbon content, for example between 0.2% and 0.5%, in particular because of a lower cost and greater wire drawability.

The metal or steel used, whether in particular a carbon steel or a stainless steel, may itself be coated with a metal layer that improves, for example, the processing properties of the metal cord and/or of its constituent components, or the usage properties of the cord and/or of the tire themselves, such as the adhesion, corrosion resistance or ageing resistance properties. According to a preferred embodiment, the steel used is coated with a layer of brass (Zn—Cu alloy) or of zinc. It will be recalled that, during the wire manufacturing process, the brass or zinc coating makes wire drawing easier and improves the bonding of the wire to the rubber. However, the wires could be coated with a thin metal layer other than a brass or zinc layer, for example having the function of improving the corrosion resistance of these wires and/or their adhesion to rubber, for example a thin layer of Co, Ni, Al, or an alloy of two or more of the compounds Cu, Zn, Al, Ni, Co, Sn.

The strands used in the multistrand cord of the invention are preferably made of carbon steel and have a tensile strength ( $R_m$ ) of preferably greater than 2500 MPa, more preferably greater than 3000 MPa. The total elongation at break (denoted by  $A_e$ ) of each constituent strand of the cord of the invention, which is the sum of its structural elastic and plastic elongations, is preferably greater than 2.0%, more preferably at least equal to 2.5%.

The elastomer (or indistinguishably "rubber", the two terms being considered as synonyms) of the filling rubber is preferably a diene elastomer, more preferably chosen from the group formed by: polybutadienes (BR); natural rubber (NR); synthetic polyisoprenes (IR); various butadiene copolymers; various isoprene copolymers; and blends of these elastomers. Such copolymers are more preferably chosen from the group formed by: butadiene-styrene (SBR) copolymers, whether these are prepared by emulsion polymerization (ESBR) or by solution polymerization (SSBR); isoprene-butadiene (BIR) copolymers; isoprene-styrene (SIR) copolymers; and isoprene-butadiene-styrene (SBIR) copolymers.

A preferred embodiment consists in using an isoprene elastomer, that is to say an isoprene homopolymer or copolymer, in other words a diene elastomer chosen from the group formed by: natural rubber (NR); synthetic polyisoprenes (IR); various isoprene copolymers; and blends of these elastomers. The isoprene elastomer is preferably natural rubber or a synthetic polyisoprene of the cis-1,4 type. Among these synthetic polyisoprenes, it is preferred to use polyisoprenes having a (% molar) content of cis-1,4 bonds greater than 90%, more preferably still greater than 98%. According to other preferred embodiments, the diene elastomer may consist, in total or in part, of another diene elastomer such as, for example, an SBR elastomer optionally blended with another elastomer, for example of the BR type.

The filling rubber may contain one or more, especially diene, elastomers, this or these possibly being used in combination with any synthetic elastomer other than a diene elastomer, or even with polymers other than elastomers.

The filling rubber is preferably crosslinkable, that is to say it comprises by definition a suitable crosslinking system enabling the composition to be crosslinked while it is being cured (i.e. while hardening and not melting). Thus, in such a

## 15

case, this rubber composition may be termed "unmeltable" because it cannot be melted by heating to any temperature whatsoever. Preferably, in the case of a diene rubber composition, this crosslinking system of the rubber sheath is a vulcanization system, i.e. based on sulphur (or a sulphur donor) and at least one vulcanization accelerator. Various known vulcanization activators may be added to this base vulcanization system. The sulphur is used preferably in an amount of between 0.5 and 10 phr, more preferably between 1 and 8 phr, and the vulcanization accelerator, for example a sulphenamide, is used preferably in an amount of between 0.5 and 10 phr, more preferably between 0.5 and 5.0 phr.

However, the invention also applies to cases in which the filling rubber contains no sulphur and even contains no other crosslinking system, given that, to crosslink it, the crosslinking or vulcanization system present in the rubber matrix that the cord of the invention is intended to reinforce, and capable of migrating, by contact with said surrounding matrix, into the filling rubber, could suffice.

The filling rubber may also include, apart from said crosslinking system, all or some of the additives normally used in rubber matrices intended for manufacturing tires, such as, for example: reinforcing fillers, such as carbon black or inorganic fillers, such as silica; coupling agents; anti-ageing agents; antioxidants; plasticizers or oil extenders, whether the latter be of aromatic or non-aromatic nature, especially oils which are very slightly aromatic or are non-aromatic, for example of the naphthenic or paraffinic type, of high or preferably low viscosity, MES or TDAE oils; plasticizing resins having a high  $T_g$  greater than 30°C.; processing aids (which make it easier to process the compositions in the uncured state); tackifying resins; antireversion agents; methylene acceptors and donors, such as for example HMT (hexamethylenetetramine) or H3M (hexamethoxymethylmelamine); reinforcing resins (such as resorcinol or bismaleimide); and known adhesion promoter systems of the metal salt type, for example, in particular cobalt, nickel or lanthanide salts, as described in particular in patent application WO 2005/113666.

The amount of reinforcing filler, for example carbon black or a reinforcing inorganic filler such as silica, is preferably greater than 50 phr, for example between 60 and 140 phr. It is more preferably greater than 70 phr, for example between 70 and 120 phr. Suitable carbon blacks are all carbon blacks, especially blacks of the HAF, ISAF, SAF type, conventionally used in tires (these being called tire-grade blacks). Among the latter, mention may more particularly be made of carbon blacks of ASTM grade 300, 600 or 700 (for example, N326, N330, N347, N375, N683 and N772). Suitable inorganic reinforcing fillers are especially mineral fillers of the silica ( $SiO_2$ ) type, in particular precipitated or fumed silicas having a BET surface area of less than 450  $m^2/g$ , preferably from 30 to 400  $m^2/g$ .

A person skilled in the art will know, in the light of the present description, how to adjust the formulation of the filling rubber so as to achieve the desired levels of properties (especially elastic modulus) and how to adapt the formulation to the specific intended application.

According to a first embodiment of the invention, the formulation of the filling rubber may be chosen to be identical to the formulation of the rubber matrix that the cord of the invention is intended to reinforce. Thus, there is no compatibility problem between the respective materials, namely the filling rubber and said rubber matrix.

According to a second embodiment of the invention, the formulation of the filling rubber may be chosen to be different from the formulation of the rubber matrix that the cord of the

## 16

invention is intended to reinforce. In particular, the formulation of the filling rubber may be adjusted using a relatively high amount of adhesion promoter, typically for example 5 to 15 phr of a metal salt, such as a cobalt salt, a nickel salt or a neodymium salt, and by advantageously reducing the amount of said promoter (or even completely eliminating it) in the surrounding rubber matrix.

Preferably, the filling rubber has, in the crosslinked state, a tensile secant modulus E10 (at 10% elongation) which is between 5 and 25 MPa, more preferably between 5 and 20 MPa, in particular in the range from 7 to 15 MPa.

A person skilled in the art will understand that the strands used in the multistrand cord of the invention described above could optionally be rubberized in situ with a filling rubber based on elastomers other than dienes, especially thermoplastic elastomers (TPEs) such as for example polyurethane (TPU) elastomers, which do not require, as is known, to be crosslinked or vulcanized but which have, at the service temperature, properties similar to those of a vulcanized diene elastomer.

However, and particularly preferably, the present invention is carried out with a filling rubber based on diene elastomers as described above, in particular using a specific manufacturing process which is particularly suitable for such elastomers, this manufacturing process being described in detail below.

## II-2. Manufacture of the Multistrand Cord of the Invention

## A) Manufacture of the Elementary Strands

The elementary strands of (L+M) construction described above, rubberized in situ preferably with a diene elastomer, can be manufactured using a specific process comprising the following steps, preferably carried out in line and continuously:

firstly, when L is different from 1, an assembly step, in which the L core wires are twisted together, to form the inner layer (C1) at an assembly point;  
then, upstream of said point where the L core wires are assembled (L differing from 1), a sheathing step in which the inner layer (C1) is sheathed with the uncured (i.e. uncrosslinked) filling rubber;  
followed by an assembly step in which the M wires of the outer layer (C2) are twisted around the inner layer (C1) thus sheathed; and  
then a final twist-balancing step.

It will be recalled here that there are two possible techniques for assembling metal wires:

either by cabling: in such a case, the wires undergo no twisting about their own axis, because of a synchronous rotation before and after the assembly point;  
or by twisting: in such a case, the wires undergo both a collective twist and an individual twist about their own axis, thereby generating an untwisting torque on each of the wires and on the cord itself.

One essential feature of the above process is the use, both for assembling the inner layer C1 and assembling the outer layer C2, of a twisting step.

In the case in which L is equal to 1, that is to say it is the single core wire that undergoes the step of being sheathed with the filling rubber in the uncured state, before the M wires of the outer layer (C2) are assembled by being twisted around the core wire thus sheathed.

During the first step, the L core wires are twisted together (S or Z direction) in order to form the inner layer C1, in a manner known per se; the wires are delivered by supply means, such as spools, a distributing grid, whether or not

coupled to an assembling guide, intended to make the core wires converge on a common twisting point (or assembly point).

The inner layer (C1) thus formed is then sheathed with uncured filling rubber, supplied by an extrusion screw at a suitable temperature. The filling rubber may thus be delivered to a single fixed point, of small volume, by means of a single extrusion head without having to individually sheath the wires upstream of the assembly operations, before formation of the inner layer as described in the prior art.

This process has the considerable advantage of not slowing down the conventional assembly process. It thus makes it possible for the complete operation—initial twisting, rubberizing and final twisting—to be carried out in line and in a single step whatever the type of strand produced (compact strand or cylindrically layered strand), all at high speed. The above process may be carried out at a speed (run speed of the strand on the twisting-rubberizing line) of greater than 70 m/min, preferably greater than 100 m/min.

Upstream of the extrusion head, the tension exerted on the L wire or wires, substantially identical from one wire to the other, is preferably between 10 and 25% of the breakage strength of the wires.

The extrusion head may comprise one or more dies, for example an upstream guiding die and a downstream sizing die. It is possible to add means for measuring and controlling the diameter of the strand continuously, these means being connected to the extruder. Preferably, the temperature at which the filling rubber compound is extruded is between 60° C. and 120° C., more preferably between 70° C. and 110° C. The extrusion head thus defines a sheathing zone having the form of a cylinder of revolution, the diameter of which is for example between 0.4 mm and 1.2 mm, and the length of which is for example between 4 and 10 mm.

The amount of filling rubber delivered by the extrusion head may be easily adjusted in such a way that, in the final L+M strand, this amount is between 5 and 40 mg, preferably between 5 and 35 mg and especially in the range from 10 to 30 mg per g of strand.

Preferably, at the outlet of the extrusion head, the inner layer C1, at any point on its periphery, is covered with a minimum thickness of filling rubber which is preferably greater than 5 µm, more preferably greater than 10 µm, for example between 10 and 50 µm.

On leaving the above sheathing step, the final assembly is carried out, during a new step, again by twisting (S or Z direction) the M wires of the outer layer (C2) around the inner layer (C1) thus sheathed. During the twisting operation, the M wires bear on the filling rubber, becoming encrusted therein. The filling rubber, moving under the pressure exerted by these outer wires, then naturally has the tendency to fill, at least partly, each of the interstices or cavities left empty by the wires, between the inner layer (C1) and the outer layer (C2).

At this stage, the L+M strand is however not yet finished: in particular its central channel, delimited by the 3 or 4 core wires when L is different from 1 or 2, is not yet filled with filling rubber, or in any case is not filled sufficiently to obtain an acceptable air impermeability.

The important step that follows consists in making the strand, thus provided with its filling rubber in the uncured state, pass through twist-balancing means in order to obtain what is called a “twist-balanced” cord (i.e. one with practically no residual twist). The term “twist-balancing” is understood here to mean, as is well known by those skilled in the art, the cancelling-out of the residual torques (or untwisting spring-back) exerted on each wire of the strand both in the inner layer and in the outer layer.

Twist-balancing tools are known to those skilled in the art of twisting. They may for example consist of “straighteners” and/or “twisters” and/or “twister-straighteners” consisting either of pulleys in the case of twisters or small-diameter rollers in the case of straighteners, over which pulleys or rollers the strand passes, in a single plane or preferably in at least two different planes.

It is assumed a posteriori that, upon passing through this balancing tool, the detwisting force acting on the L core wires, causing an at least partial reverse rotation of these wires about their axis, is sufficient to force the filling rubber in the green state (i.e. the uncrosslinked or uncured state) while still hot and relatively fluid so as to drive it from the outside towards the centre of the strand, right into the central channel formed by the L wires, finally offering the constituent strands of the multistrand cord of the invention the excellent air impermeability property that characterizes them. The straightening function, provided by the use of a straightening tool also has the advantage that the contact between the rollers of the straightener and the wires of the outer layer exert addition pressure on the filling rubber, further promoting penetration thereof into the central capillary formed by the L core wires.

In other words, the process described above exploits the rotation of the L core wires, in the to final stage of strand manufacture, in order for the filling rubber to be naturally distributed, homogeneously, into and around the inner layer (C1), while perfectly controlling the amount of filling rubber supplied. A person skilled in the art will in particular know how to adjust the arrangement and the diameter of the pulleys and/or rollers of the twist-balancing means in order to vary the intensity of the radial pressure exerted on the various wires.

Thus, unexpectedly, it proves to be possible to make the filling rubber penetrate to the very core of each strand of the multistrand cord of the invention by depositing the rubber compound downstream of the point of assembly of the L wires and not upstream, as described in the prior art, while controlling and optimizing the amount of filling rubber delivered by the use of a single extrusion head.

After this final twist-balancing step, the manufacture of the outer strand, rubberized in situ by its filling rubber in the uncured state, is completed. This strand is wound onto one or more take-up reels, for storage, before the subsequent operation of cabling the elementary strands to obtain the multi-strand cord of the invention.

Of course, this manufacturing process applies to the manufacture of compact-type outer strands (as a reminder, and by definition, those of which the layers C1 and C2 are wound with the same pitch and in the same direction) as cords of the cylindrically layered type (as a reminder, and by definition, those of which the layers C1 and C2 are wound either with different pitches, or in opposite directions, or else with different pitches and in opposite directions).

The process described above makes it possible, according to one particularly preferred embodiment, to manufacture outer strands and therefore a multistrand cord with no (or virtually no) filling rubber on their periphery. By this expression it is meant that no particle of filling rubber is visible, to the naked eye, on the periphery of each outer strand, or on the periphery of the multistrand cord of the invention. That is to say that a person skilled in the art would not know the difference, after manufacture, with the naked eye and at a distance of three meters or more, between a reel of multistrand cord according to the invention and a reel of conventional multi-strand cord, i.e. one not rubberized in situ.

An assembling and rubberizing device that can be used to implement the process described above is a device comprising, from the upstream end to the downstream end, in the direction of advance of a strand under manufacture:

- means for feeding the L core wires;
- means for assembling the L core wires, when L is different from 1, by twisting them in order to form the inner layer (C1);
- means for sheathing the inner layer (C1);
- at the outlet of the sheathing means, means for assembling the M outer wires by twisting them around the inner layer thus sheathed, in order to form the outer layer (C2);
- and
- finally, twist-balancing means.

The appended FIG. 7 shows an example of a twisting assembly device (100), of the rotating feed/rotating receiver type, which can be used for the manufacture of a strand of the cylindrically layered type (different pitches  $p_1$  and  $p_2$  and/or different twist directions of the layers C1 and C2), for example of (3+9) construction as illustrated in FIG. 1. In this device (100), feed means (110) deliver M (for example three) core wires (11) through a distributing grid (111) (axisymmetric distributor), which may or may not be coupled to an assembling guide (112), beyond which the M wires (11) converge on an assembly point or twisting point (113), in order to form the inner layer (C1).

Once formed, the inner layer C1 then passes through a sheathing zone consisting, for example, of a single extrusion head (114) through which the inner layer is intended to pass. The distance between the point of convergence (113) and the sheathing point (114) is for example between 50 cm and 1 m. The N wires (12) of the outer layer (C2), for example nine wires, delivered by feed means (120), are then assembled by being twisted around the inner layer C1 thus rubberized, progressing in the direction indicated by the arrow. The C1+C2 strand thus formed is finally collected on a rotating receiver (140) after having passed through the twist-balancing means (130) consisting for example of a straightener or a twister-straightener.

It will be recalled here that, as is well known to those skilled in the art, to manufacture a (3+9) strand of compact type (identical pitches  $p_1$  and  $p_2$  and identical twisting directions of the layers C1 and C2), a device (100) will be used which this time has a single rotating member (feeder or receiver), and not two as shown schematically by way of example in FIG. 4.

#### B) Manufacture of the Multistrand Cord

The process for manufacturing the multistrand cord of the invention is carried out, in a manner well known to those skilled in the art, by cabling or twisting the previously obtained elementary strands using cabling or twisting machines designed for assembling the strands.

When J is greater than 1, the J strands (J varying from 2 to 4) constituting the core of the cord of the invention, are preferably assembled by cabling. As already indicated previously, according to one possible preferred embodiment, the core of the multistrand cord of the invention may itself be sheathed with a filling rubber, the formulation of which may be identical to or different from the formulation of the filling rubber used for the in situ rubberizing of the K outer strands.

#### II-3. Use of the Multistrand Cord as Crown Reinforcement for a Tire

The multistrand cord of the invention may be used for reinforcing articles other than tires, for example hoses, belts, conveyor belts; advantageously, it could also be used for

reinforcing parts of tires other than their crown reinforcement, especially for the carcass reinforcement of tires for industrial vehicles.

However, as explained in the introduction of the present document, the cord of the invention is particularly intended as a tire crown reinforcement for large industrial vehicles, such as civil engineering vehicles, especially of the mining type.

To give an example, FIG. 8 shows very schematically a radial cross section through a tire with a metal crown reinforcement, which may or may not be in accordance with the invention, in this general representation.

This tire 1 comprises a crown 2 reinforced by a crown reinforcement or belt 6, two sidewalls 3 and two beads 4, each of these beads 4 being reinforced by a bead wire 5. The crown 2 is covered with a tread (not shown in this schematic figure). A carcass reinforcement 7 is wound around the two bead wires 5 in each bead 4, the turn-up 8 of this reinforcement 7 lying for example to the outside of the tire 1, which is shown here mounted on its rim 9. As is known per se, the carcass reinforcement 7 is formed by at least one ply reinforced by "radial" cords, that is to say these cords are practically parallel to one another and extend from one bead to the other so as to make an angle of between 80° and 90° with the median circumferential plane (the plane perpendicular to the rotation axis of the tire, which plane is located half-way between the two beads 4 and passes through the middle of the crown reinforcement 6).

The tire according to the invention is characterized in that its belt 6 comprises at least, as reinforcement for at least one of the belt plies, a multistrand cord according to the invention. In this belt 6 shown schematically in a very simple manner in FIG. 7, it will be understood that the multistrand cords of the invention may for example reinforce some or all of what are called the "working" belt plies. Of course, this tire 1 also includes, as is known, an inner layer of rubber compound or elastomer (usually called "inner liner") that defines the radially inner face of the tire and is intended to protect the carcass ply from the diffusion of air coming from the space inside the tire.

### III. EMBODIMENTS OF THE INVENTION

The following tests demonstrate the capability of the invention to provide multistrand cords of appreciably increased endurance, in particular when used as a tire belt, because of the excellent air impermeability property of the constituent strands of these cords.

#### III-1. Nature and Properties of the Wires and Cords Used

In the following tests, two-layer cords of 3+9 construction as shown schematically in FIG. 1, formed of fine brass-coated carbon steel wires, were used as elementary strands.

The carbon steel wires were prepared in a known manner, for example from wire stock (5 to 6 mm in diameter) which was firstly work-hardened, by rolling and/or drawing, down to an intermediate diameter close to 1 mm. The steel used for the cord C-1 according to the invention was an SHT (super high tensile) carbon steel, the carbon content of which being about 0.92% and containing about 0.2% chromium, the balance consisting of iron and the usual inevitable impurities due to the steel manufacturing process.

The wires of intermediate diameter underwent a degreasing and/or pickling treatment before their subsequent conversion. After a brass coating had been deposited on these intermediate wires, what is called a "final" work-hardening

operation was carried out on each wire (i.e. after the final patenting heat treatment), by cold-drawing it in a wet medium with a drawing lubricant for example in the form of an aqueous emulsion or dispersion.

The steel wires thus drawn have the following diameter and mechanical properties:

TABLE 1

| Steel | $\phi$ (mm) | $F_m$ (N) | $R_m$ (MPa) |
|-------|-------------|-----------|-------------|
| SHT   | 0.30        | 226       | 3200        |

These wires were then assembled in the form of two-layer strands of (3+9) construction (referenced 10 in FIG. 1), the mechanical properties of which, measured on strands extracted from a multistrand cord according to the invention (of (1+6)×(3+9) construction with a pitch  $P_K$  equal to 40 mm, as shown schematically in FIG. 2), are given in Table 2:

TABLE 2

| Strand | $p_1$ (mm) | $p_2$ (mm) | $F_m$ (daN) | $R_m$ (MPa) |
|--------|------------|------------|-------------|-------------|
| 3 + 9  | 7.5        | 15.0       | 256         | 3040        |

This strand (10) of (3+9) construction, as shown schematically in FIG. 1, is formed of 12 wires in total, all with a diameter of 0.30 mm, which were wound with different pitches and in the same twist direction (S/S) in order to obtain a strand of the cylindrically layered type. The amount of filling rubber, measured according to the method indicated above in section I-3, was 22 mg per g of strand.

To manufacture this strand, a device such as that described above and shown schematically in FIG. 7 was used. The filling rubber was a conventional rubber composition for a tire crown reinforcement. This composition was extruded at a temperature of 90° C. through a 0.700 mm sizing die.

### III-2. Air Permeability Tests

The strands of (3+9) construction manufactured above were also subjected to the air permeability test described in section I-2, carried out on strand lengths of 4 cm (equal to  $P_K$ ), measuring the volume of air (in  $\text{cm}^3$ ) passing through the strands in 1 minute (an average of 10 measurements for each strand tested).

For each strand (10) tested and for 100% of the measurements (i.e. ten specimens in ten), a rate of zero or less than 0.2  $\text{cm}^3/\text{min}$  was measured. In other words, the strands of the cords of the invention may be termed airtight along their axis and they are therefore optimally penetrated by the rubber.

Moreover, control in situ rubberized strands, of the same construction as the above strands (10), were prepared by individually sheathing either a single wire or each of the three wires of the inner layer C1. This sheathing was carried out using extrusion dies of variable diameter (320 to 410  $\mu\text{m}$ ) placed this time upstream of the point of assembly (in-line sheathing and twisting) as described in the prior art (according to the aforementioned US application 2002/160213). For strict comparison, the amount of filling rubber was also adjusted in such a way that the amount thereof (between 5 and 30 mg/g of strand, measured using the method of section I-3) in the final strands was close to that of the strands of the multistrand cord of the invention.

In the case of sheathing of a single wire, whatever the strand tested, it was found that 100% of the measurements

(i.e. 10 specimens in 10) showed an air flow rate greater than  $2 \text{ cm}^3/\text{min}$ . The measured average flow rate varied from 16 to 61  $\text{cm}^3/\text{min}$  depending on the operating conditions used, especially the diameter of the extrusion die tested. In other words, each of the above control strands tested could not be termed airtight along its longitudinal axis within the meaning of the test in section I-2.

In the case of the individual sheathing of each of the three wires, although the measured average flow rate proved in many cases to be less than  $2 \text{ cm}^3/\text{min}$ , it was observed that the strands obtained had a relatively large amount of filling rubber at their periphery, making them unsuitable for being calendered under industrial conditions.

In conclusion, thanks to the specific construction of its, 15 constituent outer strands and the excellent air impermeability that characterizes them, the multistrand cord of the invention is capable of having improved fatigue and fatigue-corrosion resistance, while meeting the usual cabling and rubberizing requirements under industrial conditions.

20 The invention claimed is:

1. A multistrand metal cord having two layers of J+K construction, which can notably be used for reinforcing tires for industrial vehicles, consisting of a core comprising J strands forming an inner layer, J varying from 1 to 4, around which core are wound, in a helix, with a helix pitch  $P_K$  of between 20 and 70 mm. K outer strands forming an outer layer around said inner layer, each outer strand:

comprising a cord having two layers of L+M construction, 30 rubberized in situ, comprising an inner layer comprised of L wires of diameter  $d_1$ , L varying from 1 to 4, and an outer layer of M wires, M being equal to or greater than 5, of diameter  $d_2$ , which are wound together in a helix with a pitch  $p_2$  around the inner layer; and

25 having the following characteristics ( $d_1$ ,  $d_2$  and  $p_2$  being expressed in mm):

$$0.10 < d_1 < 0.50;$$

$$0.10 < d_2 < 0.50;$$

$$6 < p_2 < 30;$$

35 wherein the inner layer of the outer strand is sheathed with a rubber composition called a "filling rubber";

over any length of the outer strand equal to  $P_K$ , the filling rubber is present in each of the capillaries delimited by the L wires of the inner layer and the M wires of the outer layer, and also, when L is equal to 3 or 4, in the central channel delimited by the L wires of the inner layer; and the amount of filling rubber in said outer strand is between 5 and 40 mg per g of strand.

40 2. The multistrand cord according to claim 1, wherein, in each outer strand, the following characteristics are satisfied:

$$0.15 < d_1 < 0.35;$$

$$0.15 < d_2 < 0.35.$$

45 3. The multistrand cord according to claim 1, wherein, in each outer strand,  $p_2$  is in the range from 12 to 25 mm.

4. The multistrand cord according to claim 1, wherein,  $P_K$  is in the range from 25 to 60 mm.

50 5. The multistrand cord according to claim 1, wherein,  $P_K$  satisfies the relationship:

$$1.5 \leq P_K/p_2 \leq 3.0.$$

55 6. The multistrand cord according to claim 1, wherein, in each outer strand, L is equal to 1.

60 7. The multistrand cord according to claim 6, wherein, each outer strand, L is equal to 1 and M is equal to 5, 6 or 7.

## 23

8. The multistrand cord according to claim 1, wherein, in each outer strand, L is different from 1 and the L wires of diameter  $d_1$  are helically wound with a pitch  $p_1$  satisfying the relationship:

$$20 < p_1/d_1 < 100.$$

9. The multistrand cord according to claim 1, wherein, in each outer strand, L is different from 1 and the L wires of diameter  $d_1$  are helically wound with a pitch  $p_1$  satisfying the relationships:

$$0.5 \leq p_1/p_2 \leq 1.$$

10. The multistrand cord according to claim 9, wherein, in each outer strand,  $p_1$  lies in the range from 6 to 30 mm.

11. The multistrand cord according to claim 8, wherein, in each outer strand,  $p_1$  is equal to  $p_2$ .

12. The multistrand cord according to claim 8, wherein, in each outer strand, L is equal to 2 and M is equal to 7, 8 or 9.

13. The multistrand cord according to claim 8, wherein, in each outer strand, L is equal to 3 and M is equal to 8, 9 or 10.

14. The multistrand cord according to claim 8, wherein, in each outer strand, L is equal to 4 and M is equal to 8, 9, 10 or 11.

15. The multistrand cord according to claim 1, wherein, in each outer strand, the following relationship applies:

$$0.7 \leq d_1/d_2 \leq 1.3.$$

16. The multistrand cord according to claim 1, wherein, in each outer strand, the wires of the outer layer are helically wound with the same pitch and in the same twist direction as the wires of the inner layer.

17. The multistrand cord according to claim 1, wherein, in each outer strand, the wires of the outer layer are helically wound either with a different pitch, or in a different twist direction, or with both a different pitch and a different twist direction, compared to the wires of the inner layer.

18. The multistrand cord according to claim 1, wherein, in each outer strand, the outer layer is a saturated layer.

19. The multistrand cord according to claim 1, wherein J is equal to 1 and K is equal to 5, 6, 7 or 8.

20. The multistrand cord according to claim 1, wherein J is equal to 3 and K is equal to 8, 9, 10, 11 or 12.

21. The multistrand cord according to claim 1, wherein, in each outer strand, the rubber of the filling rubber is a diene rubber.

22. The multistrand cord according to claim 21, wherein, in each outer strand, the diene elastomer of the filling rubber is chosen from the group formed by polybutadienes, natural

## 24

rubber, synthetic polyisoprenes, butadiene copolymers, isoprene copolymers and the blends of these elastomers.

23. The multistrand cord according to claim 22, wherein, in each outer strand, the diene elastomer is natural rubber.

5 24. The multistrand cord according to claim 1, wherein, in each outer strand, the amount of rubber filling compound is between 5 and 35 mg per g of strand.

10 25. The multistrand cord according to claim 1, wherein, in an air permeability test, each outer strand has an average air flow rate of less than 2 cm<sup>3</sup>/min.

15 26. The multistrand cord according to claim 1, wherein each of the J strands of the core, J varying from 1 to 4, is itself formed by a two-layer cord of L+M construction that satisfies the characteristics of the K outer strands.

20 27. The multistrand cord according to claim 26, wherein each of the J strands of the core, J varying from 1 to 4, has an identical construction to that of the outer strands.

20 28. The multistrand cord according to claim 26, wherein each of the J strands of the core, J varying from 1 to 4, has a different construction from that of the K outer strands.

25 29. The multistrand cord according to claim 26, comprising in total 6 strands, a central strand forming the core or inner layer and 5 outer strands forming the outer layer, said cord having the 1×(1+6)+5×(3+9) construction.

30 30. The multistrand cord according to claim 26, comprising in total 7 strands, a central strand forming the core or inner layer and 6 outer strands forming the outer layer, said cord having the (1+6)×(1+6) or (1+6)×(3+9) construction.

30 31. The multistrand cord according to claim 1, wherein, comprising in total 8 strands, a central strand forming the core or inner layer and 7 outer strands forming the outer layer, said cord having the 1×(3+9)+7×(1+6) construction.

35 32. The multistrand cord according to claim 1, wherein the core of the cord, which core is formed by the J strands, J varying from 1 to 4, is itself sheathed with the rubber filling compound.

33. A tire comprising a cord according to claim 1.

40 34. The multistrand cord according to claim 1, wherein  $P_K$  is in the range from 30 to 50 mm.

35 35. The multistrand according to claim 1, wherein  $P_1$  lies in the range from 6 to 25 mm.

45 36. The multistrand cord according to claim 25, wherein said average air flow rate is less than or at most equal to 0.2 cm<sup>3</sup>/min.

\* \* \* \* \*